

Aug. 31, 1937.

J. KESSLER

2,091,863

PROCESS OF MAKING COMMUTATOR BLOCKS FOR CATHODE RAY TUBES

Filed April 8, 1935



Patented Aug. 31, 1937

2,091,863

# UNITED STATES PATENT OFFICE

2,091,863

## PROCESS OF MAKING COMMUTATOR BLOCKS FOR CATHODE RAY TUBES

Jacob Kessler, Richmond Hill, N. Y.

Application April 8, 1935, Serial No. 15,324

3 Claims. (Cl. 250—27.5)

This invention relates to a process employed in the construction of cathode ray tubes, particularly of the type shown herein and shown, described and claimed in my co-pending application Serial No. 15,325, filed April 8, 1935, and entitled

5 Cathode ray tubes.

An object of the present invention is the provision of a method for constructing an important element of the cathode ray tube of my invention, said element being termed by me a commutator block.

10 The invention comprises a method whereby photo-sensitive material adapted to supply electrons when effected by light, may be deposited on the ends of the individual conductors comprising the mentioned block; if said light-sensitive material is easily oxidized the process is performed in a non-oxidizing atmosphere.

In the drawing:

20 Fig. 1 is a sectional view of apparatus employed in carrying out the process of my invention, the view showing the block within the apparatus.

Fig. 2 is a view of a cathode ray transmitter tube, partly in section, partly in elevation, and partly broken away.

25 Fig. 3 is a fragmentary elevational view of the light end of the commutator block which forms part of the tube shown in Fig. 2; and

Fig. 4 is a fragmentary longitudinal section of

30 the same block.

Referring to the drawing, and at first to Figs. 2, 3 and 4, the numeral 5 indicates an incandescent filament adapted to serve as the cathode ray source. Prongs 6 which project from base 7 of the cathode ray tube are the terminals of the filament, while a prong 8, which also projects from the base 7, is the terminal of a well-known Wehnelt control cylinder 9 which encircles the filament 5. A sealed bulb or envelope 10 is held in the base 7 and contains the parts illustrated as being therein, said bulb being evacuated of air and filled with an ionizable gas, said gas being, for example, argon at a few millimeters of mercury pressure. An electrode 12 is positioned within the tube in front of the filament 5 and has a central aperture 12a thru which the cathode rays may pass. The electrode 12 has a terminal 12b outside of the bulb 10, as shown, and is to be charged with a positive potential at, for example, three or four thousand volts, in order to give a high velocity to the cathode rays. Two pairs of deflector plates, designated respectively by the numerals 15 and 16, and positioned at right angles to each other, are also contained within the

bulb 10 and are in front of the disc 12. Each of the electrodes 15 and 16 is provided with terminals numbered respectively 15a and 16a, which terminals are exterior to the envelope or bulb. The deflector plates 15 and 16 and their operation in the cathode ray tube are well known, and are for the purpose of deflecting the cathode rays so that they may be directed to predetermined positions when charged respectively to varying potentials, the varying potentials of each pair being out of phase with the other pair, as well known.

In front of the deflector plates, and in the forward portion of the bulb 10, what I call a commutator block is positioned, and it is designated by the numeral 17, being held in spaced relation to the wall of the bulb by means of insulators 18. The block 17 has a plane front face 19 and a dished face 19a upon which latter face the cathode rays fall. The face 19a is a spherical surface so formed that all the rays may be normal to that part of the face on which they fall. The block 17 includes a plurality of straight electrical conductors 17a insulated from each other. The conductors 17a may be of any suitable material, such for example as copper wire, which has been coated with aluminum, the latter being subsequently converted into the oxide to function as insulating means, such insulation being designated by the character 17b. It is to be understood however that the ends of the conductors or wires 17a are not insulated. The forward ends of the conductors 17a, i. e., those which lie in the forward face 19, are preferably pitted to receive small masses 17c of light-sensitive material, such as sodium, for example, or other material adapted to emit electrons when acted on by light or other suitable electromagnetic waves. It is to be understood that the mentioned light-sensitive or photo-electric material lodged in the ends of the conductors comprising the block 17 are separated from each other by the insulating medium 17b which surrounds each conductor or wire.

Within the envelope 10 and three or four inches, for example, in front of the block 17 is a collector plate 20 having a terminal 21 outside of the envelope so that it may be charged to a positive potential of 100 volts, for example, from any suitable source. The mentioned plate 20 is to be charged to a potential sufficient to enable it to collect the electrons emanating from the photo-sensitive material 17c. The collector plate 20 is provided with an aperture 20a thru which an image may be thrown on the face 19 of the block 55

17, using an appropriate optical system 23 which is positioned in front of the envelope 10 and exterior thereto for the purpose of forming the image on the mentioned face.

5 The collector plate 20 being positively charged, a negative charge will be induced in the forward ends of the conductors 17a and in the photo-electric material 17c with a resultant positive charge on the rear ends of the conductors 17a, 10 which positive charge in the mentioned rear ends of the conductors 17a will be neutralized by the cathode rays, the electrons from the photo-electric material 17c then being free to be pulled by the collector plate to the latter. It 15 will be understood that the cathode ray beam falls on the conductors 17a successively, that is, on one conductor at a time, moving then to an adjacent conductor as controlled by the charged deflector plates, the electrons from the corresponding photo-electric masses being thereby successively released for collection on the accumulator or collector plate 20 with a resulting varying potential thereon. The mentioned resulting varying potential is due to the varying 20 electron emission from the photo-sensitive material in accordance with the varying intensity of light falling on the different light-sensitive masses lodged in the several conductors, it being readily understood that when an image is thrown 25 on the surface 19 of the block 17 the various masses of photo-sensitive material will be variably illuminated.

The present invention is concerned with the preparation of the block 17. Said block may be 30 made from conducting wires which have been coated with a metal, the oxide of which is an insulator. Such a metal coating may be of aluminum which may be converted into the oxide by any suitable method, as for example, the electrolytic method or by means of heat. The wires comprising the block will thereby be insulated 35 from each other.

The wires which comprise the commutator block 17, and which are from 3 to 5 mills in diameter, may be of a copper-aluminum alloy having a composition of 70 per cent copper and thirty per cent aluminum. In order to provide an insulating coating for such alloy wire, I remove from the alloy the copper which exists at 40 and adjacent the surface or periphery; this may be accomplished electrolytically by making the wire the anode in an electrolytic system provided with a cathode and with an electrolyte of copper-sulphate solution or other suitable dissolved copper salt. The outer surfaces of the wires after 45 the procedure just mentioned, consist of aluminum which is to be changed to aluminum oxide; this conversion may be effected by heat or electrolytically. If the conversion is to be effected 50 electrolytically the wires are made the anode in a system comprising a cathode and an electrolyte of sodium silicate, ammonium borate or other suitable salt, the voltage on the system being sufficient to oxidize the aluminum coating of the 55 wires.

The image ends of the wires comprising the block, that is, the ends forming the face 19 of the block, after assembly to form the latter, are pitted or roughened by any suitable process in 60 order that photo-sensitive material may be deposited on the mentioned ends of the wires and adhere thereto. The pitting or roughening may be effected by electrolysis, the latter process being employed to remove copper from the mentioned ends of the wires, which, as above stated, 65

may be made of a copper-aluminum alloy, it being understood that the block is made the anode in an electrolytic system similar to that used for the removal of copper from the wires at and adjacent their peripheries. The wires of the block 70 may be made of an alloy, one constituent of which is a metal whose oxide is an insulator.

The commutator block, which is provided with a band 17d extending beyond the face 19 thereof, is then placed in a casing 35 and the casing with the block therein is positioned on a support 36 within a container 37, as shown in Fig. 1. It will be noted that the image face 19 of the block 17 is uppermost in the casing 35, the rim of the latter extending about one-eighth of an inch above the upper face of the block. A tube 38 in which sodium may be vaporized and thru which sodium vapor may pass and be deposited on the upper face of the block 17, is sealed into one end of the container 37 intermediate its ends and extends from the outside to the inside of said container, the inner end of said tube being turned downwardly and positioned above the block 17. A tube 40 thru which petroleum burning oil may be passed and be delivered onto the block 17 after the sodium has been deposited thereon is also sealed into the container 37, being positioned vertically and over the block 17. A further tube 41 is also sealed into one end of the container 37 and is provided to admit hydrogen into the container.

After the block 17, together with the casing 35 in which it is contained, has been placed in the container 37, the air is evacuated from the container 37 thru an exhaust passageway 42. The mentioned container is then flushed only or more than once with hydrogen to remove the residual air, the hydrogen being admitted thru the tube 41, and the container is then filled with hydrogen at a few millimeters of mercury pressure and is then sealed therein. Sodium vapor is then passed thru the tube 38 until a layer of the same is deposited on the face 19 of the block 17. Petroleum burning oil is then admitted into the container 37 thru the tube 40 to cover the deposit of sodium existing on the block 17. The mentioned block, together with the casing 35 in which it is contained, is then removed, coated and covered face up, from the container 37 and is immersed, in similar position, in a bath of petroleum burning oil which may be heated to 92° C. to soften the sodium. While the block is in the mentioned bath of petroleum burning oil, the excess sodium is scraped off, preferably with fine steel wool less than 1 mill in diameter so that no sodium remains on the insulation existing around the individual wires comprising the block. The block is then taken out of the oil bath and put into a bath of petroleum ether, 75° to 80° C., B. P., to be thoroughly washed. The block is then taken out of the bath of petroleum ether with some of the latter covering the sodium and is placed image face up in the cathode ray tube shown in Fig. 2, this tube however being positioned vertically with its base lowermost. It will thus be seen that the deposit of sodium on the block is never exposed to the atmosphere and thus is not in danger of being oxidized. All possible care should be taken not to oxidize the sodium and to that end the mentioned oils should be freshly distilled so as to be free of oxygen.

The bulb or envelope 10 of the cathode ray tube is then exhausted of air thru a suitable opening 45 and is then flushed with hydrogen 75

which may be admitted thru the mentioned opening. The current of hydrogen evaporates the petroleum ether from the image face of the block. Hydrogen at a few millimeters of mercury pressure may then be admitted to the tube. A glow discharge is then passed thru the tube using the filament 5 and the collector plate 20 as terminals of the discharge. The hydrogen is then blown out and the tube filled with argon at a few millimeters of mercury pressure, the argon being sealed therein and functioning as a permanent ionizable medium which is to be acted on by the cathode beam and by the photo-electrons from the image surface of the block, it being understood that the passageway 45 is sealed as the tube is filled with argon.

What is claimed as new is:

1. The method of preparing a commutator block for a cathode ray tube, which block includes a bundle of insulated conducting wires, said method comprising depositing on corresponding ends of said wires a light-sensitive material adapted to emit electrons when acted on by light, the deposition of said material being performed in a non-oxidizing environment, covering said light-sensitive material with a protective coating, placing the block, with said protective coating thereon, in a cathode ray tube, removing said coating in a non-oxidizing environment, 5

2. The method of preparing a commutator block for a cathode ray tube, which block includes a bundle of insulated conducting wires, said method comprising depositing on corresponding ends of said wires a light-sensitive material adapted to emit electrons when acted on by light, the deposition of said material being performed in a non-oxidizing environment, covering said light-sensitive material with a protective coating, placing the block, with said protective coating 10 thereon, in a cathode ray tube, removing said coating in a non-oxidizing environment, and sending an electric discharge thru said tube.

3. The method of preparing a commutator block for a cathode ray tube, which block includes a bundle of insulated conducting wires, said method comprising depositing on corresponding ends of said wires a light-sensitive material adapted to emit electrons when acted on by light, the deposition of said material being 15 performed in a non-oxidizing environment, covering said light-sensitive material with a protective coating, placing the block, with said protective coating thereon, in a cathode ray tube, removing said coating in a non-oxidizing environment, sending an electric discharge thru a 20 non-oxidizing gas within said tube, removing said gas and filling said tube with a gas to be 25 permanently sealed therein.

JACOB KESSLER. 30